# EUROPEAN PATENT SPECIFICATION

(11) **EP 0 042 759 B1**
(45) Date of publication and mention of the grant of the patent: **20.02.1985**
(21) Application number: 81302819.8
(22) Date of filing: 23.06.1981
(51) Int. Cl.: B05D 3/00, B05D 7/06

(54) **Process for powder coating substrates**
Verfahren zum Pulverbeschichten von Gegenständen
Procédé pour le revêtement, par poudre, de substrats

(30) Priority: 24.06.1980 GB 8020651
(43) Date of publication of application: 30.12.1981
(73) Proprietor: Sonneborn & Rieck Ltd., Ilford Essex (GB)
(72) Inventor: Bassett, Eric Aloysious, Staines Middlesex (GB)
(74) Representative: Votier, Sidney David

## Description

The present invention relates to a processor for painting by powder coating substrates and to substrates when so coated.

Continuing increases in the cost of raw materials, and in particular oil-based solvents have increased the importance of powder coating processes (which dispense with carriers and solvents) relative to conventional paint coating (in which a considerable proportion of solvent is merely evaporated-off and lost during drying).

Where the substrate is a poor electrostatic conductor, such as wood, powder coating has been difficult to apply electrostatically without the presence of an extra conductive layer of resin base. Further, extensive heating of wood, as in an oven, dries out the wood and can give rise to an 'orange peer effect which consumers may find unappealing in certain contexts. If the substrate is metallic and flat, powder coating again has tended to produce an 'orange peel' effect.

According to the present invention we provide a process for painting by powder coating a substrate comprising applying a dry curable coating powder to a dry uncoated substrate which is either a self-supporting panel or can be divided into such a panel and heat-curing the coating, characterised in that the coating is confined by applying firmly thereto a treatment surface which does not adhere to the coating and is heat-stable up to the curing temperature of the coating powder, and heat-curing the coating whilst so confined. Depending on the nature of the treatment surface gloss or satin finish, a specifically textured finish, or other finish, may be applied to be substrate.

The treatment surface may be a roller or heated band of platen having a non-stick surface but is preferably a heat-resistant release film applied by the platen of a press. Mylar has been found to be particularly suitable as a release film. As indicated previously, an appropriate surface of the release film gives a corresponding surface to the final coating; thus satin finish Mylar would give a satin final finish and gloss finish Mylar would give a gloss final finish. Further a suitable treatment surface on the release film or platen, roller or heated band would be used to apply texture, such as wood- grain or cloth weave texture, to the final coating.

The substrate may be any material which is in the form of a self-supporting panel or can be divided into such a panel and to which a powder coating would be applied as a surface coating layer, but it is particularly preferred to apply the process of the present invention to the coating of man made fibre or particle boards such as chipboard or hardboard.

Examples of suitable heating cycles would be 3 minutes at 180°C where the coating powder is an expoxy-polyester and 10 minutes at 180°C where the coating is a polyester/poly- urethane; although shorter heating times are desirably used. Although a wide range of pressures may be used, the pressure employed would normally only be light and just sufficient pressure to slightly squash the coating surface during fusing is generally adequate.

A thickness of powder coating in the region of 35 to 75 µ has been found to be satisfactory, although a somewhat thicker or thinner coating may be used if desired.

The process of the present invention will now be illustrated with reference to the accompanying drawings, in which:
Figure 1 shows diagrammatically one embodiment of a process according to the present invention,
Figure 2 shows diagrammatically an alternative embodiment of a process according to the present invention, and
Figure 3 shows diagrammatically a further embodiment of a process according to the present invention.

A substrate 1, which is in this instance a chipboard panel has applied thereto powder coating 2 by a spray or blade curtain coating ,apparatus, at station A, D or G.

As shown in Figure 1, the coated board 1 is then transported to station B where it is supported between the upper and lower portions 9 and 8 of a platen press. A surface of heat resistant release film 5, which is of Mylar, is interposed between the upper portion 9 of the platen press, and the powder 2 previously applied to board 1. Pressure and heat is then applied by the platen press; the time and temperature being determined by the powder type used. When the powder has cured, the board 1 having a smooth or suitably textured surface 3 is transported to station C.

In the embodiment of Figure 2, the coated board from station D is transported to station E and is passed through a heated roller press comprising rollers 11 and 12. Roller 11 is heated and has its surface covered with a Mylar release film 5. The pressure, temperature and speed of transport through the roller press are again adjusted to be appropriate to the powder type used. The finished board 1 having the desired surface 3 is thereafter transported to station F.

In the process shown in Figure 3, the so- called hot-band system, the coated board from station G is transported to station H where it is passed beneath a conventional heated band apparatus, comprising a heated band 19 passing around rollers 13 and 15. The heated band 19 may carry a layer of heat-resistant release film on its outer surface or may have an appropriate non-stick outer surface coating. An appropriate heat source 17 within heated band 19 is provided for curing powder 2. As in the embodiment of Figure 2, the pressure, temperature and speed of transport are adjusted to be appropriate to the powder type used. The finished board 1 having the desired surface 3 is thereafter transported to station /.

The hot band system has the greatest potential for large production quantities and is therefore preferred where coated boards are to be mass produced.

## Claims

1. A process for painting by powder coating a substrate surface comprising applying a dry heat-curable coating powder paint to a dry uncoated substrate which is either a self-supporting panel or can be divided into such a panel, and heat-curing the coating, characterised in that the coating is confined by applying firmly thereto a treatment surface which does not adhere to the coating and is heat-stable up to the curing temperature of the heat-curable coating powder paint, and that the coating is heat-cured whilst so confined.

2. A process according to claim 1 in which the uncoated substrate is chipboard or hardboard.

3. A process according to claim 1 or 2 in which the treatment surface is provided by a layer of heat-resistant release film.

4. A process according to any of the foregoing claims in which heat and pressure are applied for curing by a platen press.

5. A process according to any of claims 1 to 3 in which heat and pressure are applied for curing by a heated band.

6. A process according to any of the foregoing claims in which the treatment surface carries a texture.

## Patentansprüche

1. Verfahren zum Färben einer Substratoberfläche durch Pulverbeschichtung unter Aufbringung eines trockenen hitzehärtbaren Beschichtungsfarbpulvers auf ein trockenes unbeschichtetes Substrat, das entweder aus einer selbsttragenden Platte besteht oder in eine solche zerlegt werden kann, und Hitzehärtung des Beschichtung, dadurch gekennzeichnet, daß die Beschichttung eingeschlossen wird durch festes Anlegen einer Behandlungsfläche, die nicht an der Beschichtung haftet und bis zur Härtungstemperatur des hitzehärtbaren Beschichtungsfarbpulvers hitzebeständig ist, und daß die Beschichtung in derart eingeschlossenem Zustand hitzegehärtet wird.

2. Verfahren nach Anspruch 1, bei welchem das unbeschichtete Substrat aus einer Spanplatte oder Hartfaserplatte besteht.

3. Verfahren nach Anspruch 1 oder 2, bei welchem die Behandlungsfläche aus einer Schicht einer hitzebeständigen Trennmittelfolie besteht.

4. Verfahren nach einem der vorfergehenden Ansprüche, bei welchem Hitze und Druck zum Härten durch eine Plattenpresse aufgebracht werden.

5. Verfahren nach einem der Ansprüche 1 bis 3, bei welchem Hitze und Druck zum Härten durch ein geheiztes Band aufgebracht werden.

6. Verfahren nach einem der vorhergehenden Ansprüche, bei welchem die Behandlungsfläche eine Texturierung aufweist.

## Revendications

1. Un procédé pour peindre la surface d'un substrat à partir d'une couche de poudre, en appliquant à secue couche de poudre adaptée à être traitée à chaud, sur un substrat sec et nu constitué par un panneau auto-porteur ou pouvant être réduit à un tel panneau, et en traitant ensuite à chaud cette couche de poudre, caractérisé en ce qu'on soumet cette couche à un confinement, en y appliquant de manière ferme une surface de traitement qui n'adhère pas à la couche, et quie conserve sa stabilité à chaud, jusqu'à la température de traitement de la couche de poudre; et en ce qu'on effectue le traitement à chaud de la couche pendant qu'elle est ainsi confinée.

2. Un procédé selon la revendication 1, dans laquelle le substrat nu est constitué par un panneau de particules, ou un panneau en fibres.

3. Un procédé selon la revendication 1 ou 2, dans laquelle la surface de traitement est pourvue d'une couche de décollement, constituée par un film résistant à la chaleur.

4. Un procédé selon l'une quelconque des revendications 1 à 3, dans laquelle on applique la chaleur et la pression d'appui du traitement au moyen d'une presse à plateaux.

5. Un procédé selon l'une quelconque des revendications 1 à 3, dans laquelle on applique la chaleur et la pression pour durcissement au moyen d'une bande chauffante.

6. Un procédé selon l'une quelconque des revendications précédentes, caractérisé en ce que la surface de traitement porte une texture.
